

# UNITED STATES PATENT OFFICE.

GODFREY STEERUP, OF CHICAGO, ILLINOIS, ASSIGNOR TO U. S. LIGHT & HEAT CORPORATION, OF NIAGARA FALLS, NEW YORK, A CORPORATION OF NEW YORK.

## STORAGE-BATTERY SEPARATOR

1,370,064.

Specification of Letters Patent. Patented Mar. 1, 1921.

No Drawing.

Application filed June 7, 1919. Serial No. 302,595.

To all whom it may concern:

Be it known that I, GODFREY STEERUP, a citizen of the United States, residing at Chicago, in the county of Cook and State of Illinois, have invented new and useful Improvements in Storage-Battery Separators, of which the following is a specification.

The present invention relates to storage battery separators.

Storage battery separators have been manufactured of a great variety of materials. One material which is commonly used for this purpose is wood, but most varieties of wood contain plate-destroying constituents which should be removed or at least, greatly reduced in amount before the wood may be used for storage battery separators. Various processes have been devised for removing these undesirable constituents, most of which processes leave the wood in a weakened condition, whereby in service the separators break down and cause a great deal of trouble and expense.

An object of the present invention is to provide an improved method of treating wood to prepare the same for storage battery separators.

A further object is to provide a commercial process for preparing wood for storage battery separators which will result in the practical elimination of substances which are injurious in service or the changing of said substances to innocuous substances and which will leave the structure of the wood in good condition.

A further object is to provide a method of preparing wood separators which will be tougher and sturdier than those at present in use.

Further objects will be apparent as the description proceeds.

A description of the present invention may be prefaced by the statement that a steam treatment will have an effect of eliminating certain of the plate-destroying constituents from the wood. This steam treatment may be at a moderate temperature for a relatively long period of time, or at a higher temperature for a shorter period of time. However, if either of these steam treatments is conducted in the presence of a substantial amount of either alkali or acid, the action on the wood is highly detrimental. In view of the fact that the action of steam at high temperatures in raw wood

will result in the generation of acid, the wood must be given a preliminary treatment.

According to the present invention, sheets of wood cut into approximately the size required for separators, are moistened with water by capillarity. After the water has permeated the cells of the wood, the separators are placed in an autoclave and heated with live steam at a moderate temperature. This steam treatment may be conducted with a slight continuous escape of steam or steam may be let off at intervals. This steam treatment at the moderate temperature which is to be chosen at a value such that in a short period of time it will not have a detrimental action on the wood, will open the pores of the wood and will also change acid-forming constituents into free acid to a certain extent.

After the separators have been given the preliminary steam treatment above referred to, they are treated with a volatile agent capable of reacting chemically upon constituents of the wood which would prove injurious in service. For this purpose I prefer to use a volatile nitrogenous agent, such as ammonia.

In order that the volatile agent may permeate the pores of the wood, it is preferable first to reduce the pressure within the autoclave to a high state of vacuum. The volatile agent ammonia, in a gaseous state, is then allowed to surround the separators, preferably under pressure, whereby said ammonia will permeate to the innermost cells of the separators, effectually neutralizing any acidity of the wood.

After treating with ammonia for a period sufficient to effectually permeate the wood, the operator will turn on the steam at approximately the same temperature as was used in the preliminary steam treatment, a slight escape of steam being permitted whereby to allow the escape of the ammonia, thereby leaving the wood in a neutral condition or only slightly alkaline, alkalinity being preferable to acidity during the next step of the process.

After the wood has been rendered neutral, or only slightly alkaline, it is in the proper condition to receive a steam treatment at a higher temperature, without detriment. Such a treatment at a higher temperature is now given, which temperature may be chosen at a value which would injure the

structure of the wood if it had not been given the treatment described above. During the treatment following the ammonia treatment, or during the treatment at the higher temperature, or during both these periods, there will occur a volatilization of the acid-forming constituents in the form of ammonia or other compounds. For this purpose, the steam treatments may be conducted with a slight escape of steam. The treatment at the higher temperature may be continued until the bulk of the ammonium compounds are volatilized. The proper length of time and temperature for this treatment may be readily determined for each of the different varieties of wood.

After the treatment at the higher temperature, it is advisable to give a finishing treatment at a lower temperature, which may be chosen substantially equal to that in the preliminary steam treatment above referred to. This finishing treatment will volatilize the small quantity of ammonium compounds still remaining in the pores of the wood but will not result in starting any new cycles of transformation of parts of the wood not hitherto acted upon. The plate corroding elements which will remain in the wood will be so small in amount as to have no appreciable effect in service.

As a precautionary step, the finishing treatment may be supplemented by a short vacuum treatment to eliminate volatile substances that may lie in the pores of the wood.

Referring to specific figures which I have found to be practicable, but which are given for illustration only, the initial moistening has been accomplished by allowing 500 separators of bass or poplar of a standard size,  $5\frac{1}{2}$  by  $5\frac{1}{2}$  inches, to absorb twelve pints of water by capillarity. This process has been allowed to continue for twenty-four hours. The separators are then placed in an autoclave and heated with live steam to a temperature of  $255^{\circ}$  F. for a period of from four to seven hours, this step constituting the preliminary steam treatment referred to above. The steam is then blown off and by means of a vacuum pump, the pressure is reduced to 26 inches of vacuum. Preferably 28 ounces of anhydrous ammonia are introduced into the autoclave of approximately four cubic feet capacity under pressure, said ammonia being allowed to permeate the pores of the wood for approximately ten hours. The steam is then turned on again and the treatment at  $255^{\circ}$  F. continued for three hours, after which the steam is blown off, thereby purifying the wood by elimination of volatile constituents and leaving the same practically neutral, or only slightly alkaline. The steam is then turned on again and the treatment continued at a temperature of 270 F. for three

hours, the steam being blown off entirely at the end of the first one and one half hours and again at the end of three hours. The finishing treatment is then given with steam at  $255^{\circ}$  F. for a period of two hours, after which the steam is again blown off. A vacuum pump then operates to produce a high vacuum for approximately ten minutes, thus eliminating volatile substances that may lie in the pores of the wood. It will be understood that each of the steam treatments above referred to will preferably be conducted with a slight escape of steam.

The resulting separators are tough, stand up well in service and their use does not affect the plates adversely.

It is to be understood that no hard and fast rules for treating all of the varieties of wood can be set down in this specification. The treatment will vary greatly with different varieties, particularly in the temperatures involved and the length of time required for the various steps. The description which has been given is intended to set forth the steps whereby the wood may be put in such condition that its use will not affect the plates adversely.

Many modifications will occur to those skilled in the art. It is intended that this patent shall cover all such modifications that fall within the scope of the invention as defined by the appended claims.

What I claim as new and desire to secure by Letters Patent of the United States, is—

1. The method of manufacturing separators which consists in treating wood with ammonia for the purpose of conditioning said wood, volatilizing the free ammonia and its compounds and treating with steam at a temperature which would injure the structure of the raw wood.

2. The method of manufacturing separators which consists in treating raw wood with steam at a temperature and for a period of time insufficient to injure the cellular structure of the wood, treating with ammonia to condition the wood to safely receive steam treatment which would injure raw wood, treating with steam to volatilize free ammonia and its compounds, treating with steam at a temperature and for a period of time sufficient to injure raw wood and volatilizing residual ammonium compounds with steam at a lower temperature.

3. The method of manufacturing separators which consists in moistening wood with water, treating said wood with steam at a temperature and for a period of time insufficient to injure the cellular structure of the wood, treating with ammonia to condition the wood to safely receive steam treatment which would injure raw wood, treating with steam to volatilize free ammonia and its compounds, treating with steam at a temperature and for a period of time sufficient

to injure raw wood and volatilizing residual ammonium compounds with steam and vacuum at a lower temperature.

4. The method of manufacturing separators which consists in treating raw wood with steam at a temperature insufficient to injure the cellular structure of said wood, treating with ammonia, volatilizing the free ammonia and its compounds and treating with steam at a temperature and for a period of time which would injure raw wood.

5. The method of preparing separators which consists in treating wood with a volatile agent capable of rendering the wood innocuous to battery plates.

6. The method of preparing separators which consists in treating wood with a volatile nitrogenous agent capable of rendering the wood innocuous to battery plates.

20 7. The method of preparing separators which consists in treating wood with a volatile ammoniacal agent capable of rendering the wood innocuous to battery plates.

25 8. The method of preparing separators which consists in treating wood to open the pores of same, impregnating with ammonia

in gaseous form, volatilizing the free ammonia and its compounds and treating with steam at a temperature and for a length of time which would injure the cellular structure of the wood in untreated condition. 30

9. The method of preparing separators which consists in treating wood to open the pores of same, impregnating with ammonia, volatilizing the free ammonia and its compounds and treating with steam. 35

10. The method of manufacturing separators which consists in moistening wood, treating with steam at a moderate temperature, treating with ammonia in gaseous form, purifying with steam at moderate temperature to volatilize the free ammonia, treating with steam at a temperature and for a period of time which would injure the structure of raw wood, giving a finishing steam treatment at a moderate temperature and subjecting the wood to a vacuum treatment to insure the elimination of all volatile substances. 40 45

In witness whereof, I have hereunto subscribed my name. 50

GODFREY STEERUP.